

## UNITED STATES PATENT OFFICE

ARNOLD DOSER, OF COLOGNE-MULHEIM, GUSTAV MAUTHE, OF COLOGNE-HOLWEIDE,  
AND ALFRED THAUSS, OF COLOGNE-DEUTZ, GERMANY, ASSIGNORS TO GENERAL  
ANILINE WORKS, INC., OF NEW YORK, N. Y., A CORPORATION OF DELAWARE

## TREATMENT OF ANIMAL FIBERS AND PRODUCT THEREOF

No Drawing. Application filed January 19, 1929, Serial No. 333,742, and in Germany January 25, 1928.

Our present invention relates to a process of subjecting animal fibers to the action of resist compounds having the property of preventing the animal fibers from taking up substantive dyestuffs, more particularly it relates to a process which comprises incorporating with animal fibers a water soluble product being obtainable by reacting with an aralkyl halogenide upon a compound of the group comprising recent resins (for instance resins of acid character, such as colophony, shellac and the like) and condensation products of the resins with phenols in the presence of a suitable dehydrating agent, such as zinc chloride, at a temperature between about 100-200° C., and sulfonating the products thus obtainable. 5

We have found that these products, or also the corresponding products from mixtures of recent resins of different origin, possess in the free form as well as in the form of their alkali metal salts the valuable technical property of preventing animal fibers, such as wool, silk and the like, from the taking up of substantive dyestuffs. The incorporating of our resists with animal fibers may be performed from their neutral or weakly acid or alkaline aqueous solutions, advantageously in the manner of a dyeing 10 process. In this latter case, especially for the production of multi color effects in mixed textile fabrics, made for instance of wool and cotton or of silk and cotton and the like, it is possible to combine the process of applying the resists to the fibers with the dyeing process; the wool or the silk are in all these cases protected against the taking up of substantive dyestuffs to a far reaching extent. 15

40 The following examples illustrate our invention, without limiting it thereto:—

*Example 1.*—In a mixed fabric of cotton and wool the latter is dyed with 1% of orange II (Schultz, Farbstofftabellen 1923, I. page 55, No. 145) with the addition of 10% of sodium sulfate and of 3% of sulfuric acid. The fabric is then introduced into a bath containing 2% of brilliant benzo blue 6 B (Schultz, Farbstofftabellen 1923, I. page 135, No. 424) and 30% of sodium

sulfate, to which are also added 5% of the sodium salt of the sulfonic acid, obtainable by reacting with 3 parts of benzylchloride in the presence of 0.2 parts of zinc-chloride and at a temperature of about 110° to 120° C. upon 10 parts of the condensation product prepared by heating a mixture of 30 parts of colophony and 10 parts of phenol with 1.5 parts of sulfuric acid of 60° Bé at a temperature of about 70° to 80° C. for about 8 hours, until the evolution of gas has ceased, and sulfonating the condensation product with 2 parts of a 100% sulfuric acid. The fabric is left in this base for 1 hour at 50° C. The substantive dyestuff leaves the wool almost uncolored. 55

*Example 2.*—The dyeing of the wool is carried out as in Example 1, but there are added in this case to the dye bath solution of the substantive dyestuff 5% of the sodium salt of the sulfonic acid, obtainable by heating 150 parts of colophony and 50 parts of phenol to about 70° C., adding then 2 parts of sulfuric acid of 60° Bé, raising the temperature to 110° C., adding 1.5 parts of zinc chloride and 67 parts of benzylchloride and keeping the reaction mixture at a temperature of about 110° to 120° C. until the development of gas has ceased, and finally sulfonating the product by removing the water formed, mixing with 200 parts of tetrachloroethane at 70° C., gradually adding 150 parts of sulfuric acid of 100% strength, whereby the temperature is slowly lowered to 45° C. and stirring the melt for some hours at this temperature. The wool is even less colored as in Example 1. 70 75 80 85

We claim:—

1. The process which comprises incorporating with animal fibers a product being obtainable by reacting with an aralkyl halogenide upon a compound of the group comprising recent resins and condensation products of recent resins with phenols, in the presence of zinc chloride at a temperature between about 100-200° C., and sulfonating the product thus obtainable. 90

2. Animal fibers having incorporated therewith a product being obtainable by reacting with an aralkyl halogenide upon a 100

compound of the group comprising recent resins and condensation products of recent resins with phenols, in the presence of zinc chloride at a temperature between about 5 100-200° C., and sulfonating the product thus obtainable.

3. The process which comprises incorporating with animal fibers a product obtainable by reacting with benzylchloride upon 10 the condensation product prepared from colophony and phenol in the presence of zinc chloride at a temperature of 110° to 120° C., and sulfonating the product thus obtainable.
- 15 4. Animal fibers having incorporated therewith a product obtainable by reacting with benzylchloride upon the condensation product prepared from colophony and phenol in the presence of zinc chloride at a 20 temperature of 110° to 120° C., and sulfonating the product thus obtainable.

In testimony whereof we have hereunto set our hands.

ARNOLD DOSER. [L. S.]  
25 GUSTAV MAUTHE. [L. S.]  
ALFRED THAUSS. [L. S.]

30

35

40

45

50

55

60

65